

1

3,456,791

SEPARATION OF SCHOENITE BY FLOTATION  
Jose L. Ramirez, Agro-Quimicas de Honduras, Apartado  
Postal 362, Tegucigalpa, Honduras  
No Drawing. Filed Apr. 17, 1967, Ser. No. 631,180  
Int. Cl. B03d 1/02  
U.S. Cl. 209—166

5 Claims

ABSTRACT OF THE DISCLOSURE

A froth flotation process for separating schoenite from salt mixtures containing schoenite in admixture with other salts, such as sodium chloride, magnesium sulfate hydrates and kainite, in which the flotation agent is a collector in the form of a water-soluble petroleum sulfonate having a molecular weight between 300 and 400.

BACKGROUND OF THE INVENTION

Field of the invention

This invention relates to the concentration and separation of schoenite from salt mixtures containing sodium chloride, epsomite and other impurities in the medium of an aqueous brine by froth flotation to obtain schoenite 25 concentrates of high purity and with high yields from the raw salt mixtures.

Description of the prior art

The separation of schoenite (commonly represented as  $K_2SO_4 \cdot MgSO_4 \cdot 6H_2O$ ) from salt, epsomite and other impurities by flotation procedures has heretofore been disclosed, as shown, for instance, in German Patent No. 945,622; Italian Patent No. 573,975; and in J. Applied Chem. (USSR), 12, 836 (1939), various flotation agents having been suggested including alkyl sulfates, saturated and unsaturated fatty acids, naphthenic acid, and sulfo-naphthenic acid. Generally, these agents require, for their reasonably effective use, the addition of various dispersants and frothers.

SUMMARY OF THE INVENTION

My invention provides a simpler and less costly separation procedure utilizing certain petroleum sulfonates, generally without the need for dispersants and frothers. Sulfonated petroleum oils with a molecular weight of from 300 to 400, and which are water-soluble, and are used in the form of their water-soluble salts, notably their sodium salts, have been found to be very effective. A typical flotation agent consists, in commercial form, of the order of 30% petroleum sulfonates, 50% water, 10% mineral oil and 10% inorganic salts. The flotation agent may, of course, be used in a more purified, active form but this is unnecessary. While the invention is particularly useful in processing schoenite produced by the conversion of kainite to schoenite, it is also applicable to any salt mixture containing schoenite and one or more of kainite (commonly represented as  $KCl \cdot MgSO_4 \cdot 2.75H_2O$ ), sodium chloride, epsomite (commonly represented as

$MgSO_4 \cdot 7H_2O$ )

and other impurities. My invention will be described below in connection with schoenite obtained from the conversion of kainite, but it will be understood that it is not limited thereto.

DESCRIPTION OF THE PREFERRED  
EMBODIMENTS

In the practice of my invention, generally speaking, a raw salt mixture, which typically may contain of the order of 25% schoenite, 50% sodium chloride, 12% epsomite, 12% kainite, and including minor amounts of

2

other impurities, is slurried with a kainite-schoenite conversion end liquor, typically containing of the order of 8% sodium chloride, 4% potassium chloride, 8% magnesium chloride, 11% magnesium sulfate, and the balance water. The slurry which is conditioned with the petroleum sulfonate flotation agent, and which may be diluted with additional kainite-schoenite conversion end liquor, is then treated in a flotation cell. When air is introduced to the flotation cell, a froth containing mainly schoenite is formed and removed from the cell.

Contrary to many other procedures, only the aforesaid petroleum sulfonate flotation agent is added to the slurry, and, although frothers and depressants may be used, they are generally not necessary. Frequently, the presence of clay or other fine particles in the raw salts makes effective flotation very difficult. With the petroleum sulfonate flotation agent, a schoenite float of good purity may be obtained even in the presence of appreciable amounts of clay.

The application of my invention may be further understood by the following illustrative examples. All percentages recited are by weight.

Example 1

Salts from the conversion of crude kainite to schoenite were slurried as a 50% slurry with a kainite-schoenite conversion liquor. The composition of the solids, which contain about 24% schoenite, 52% sodium chloride, 12% epsomite and 12% kainite, and the liquor are shown in Table 1.

TABLE I

|             | Analysis, percent |      |      |       |        |        |
|-------------|-------------------|------|------|-------|--------|--------|
|             | K                 | Na   | Mg   | Cl    | $SO_4$ | $H_2O$ |
| Feed solid  | 5.98              | 20.0 | 3.48 | 32.20 | 19.20  | 19.14  |
| Feed liquor | 1.82              | 3.15 | 4.12 | 12.20 | 9.00   | 69.71  |

A sulfonated petroleum oil flotation agent, in this example "Petrofloe 130," (Witco Chemical Company) and containing about 30% water-soluble petroleum sulfonates, with molecular weight between about 350 and 370, together with 50% water, 10% mineral oil and 10% inorganic salts was added in the proportion of 600 grams of agent per metric ton of solid feed, and the slurry with reagent was conditioned for about 5 minutes. The slurry was diluted to 25% solids by the addition of kainite-schoenite conversion liquor, and placed in a flotation cell. When air was introduced into the agitated flotation cell, a froth containing schoenite formed at the top of the cell. This float was removed and weighed, and the residue salts were also removed. Compositions of the float and residue are shown in Table II.

TABLE II

|         | Analysis, percent |       |      |       |        |        |
|---------|-------------------|-------|------|-------|--------|--------|
|         | K                 | Na    | Mg   | Cl    | $SO_4$ | $H_2O$ |
| Float   | 16.51             | 2.41  | 5.33 | 5.27  | 39.86  | 30.52  |
| Residue | 1.47              | 34.09 | 0.64 | 53.54 | 3.13   | 7.13   |

The float, weighing 239 grams, containing about 92% schoenite and 7.3% sodium chloride, represented a yield of about 86% of the schoenite in the feed salts.

Example 2

Feed salts similar to those of Example 1, but containing an appreciable amount of clay, were floated. The feed salts and feed liquor, whose compositions are essentially those given in Table I of Example 1, were slurried as a 50% slurry, and after 600 grams per metric ton of petroleum sulfonate reagent was added, were conditioned for about 5 minutes. Kainite-schoenite conversion liquor was added to dilute the slurry to 25% solids, and the slurry was placed in a flotation cell. With the introduction of air to

the flotation cell, a froth containing schoenite was formed and removed from the cell. Compositions of the float and residue are shown in Table III.

TABLE III

|         | Analysis, percent |       |      |       |                 |                  |
|---------|-------------------|-------|------|-------|-----------------|------------------|
|         | K                 | Na    | Mg   | Cl    | SO <sub>4</sub> | H <sub>2</sub> O |
| Float   | 16.41             | 1.45  | 5.76 | 2.83  | 39.54           | 34.00            |
| Residue | 4.26              | 22.79 | 2.19 | 37.78 | 12.25           | 20.73            |

The float, weighing 149 grams, contained about 97% schoenite and 2.8% sodium chloride, and represented a yield of about 53% of the schoenite in the feed salts.

## Example 3

The yield from the flotation may be increased by refloating the residue salts, without additional reagent consumption. Feed salts identical to those of Example 1 were ground to -32 mesh and conditioned for about 5 minutes as a 50% slurry in kainite-schoenite conversion liquor with 400 grams of petroleum sulfonate reagent per metric ton of solids. The slurry was diluted to 25% solids with kainite-schoenite conversion liquor and placed in a flotation cell. The froth produced when air was introduced to the cell was removed, and the residue was also removed and reconditioned for 20 minutes with an additional 200 grams of petroleum sulfonate reagent per metric ton of solids.

The residue was refloated, and another schoenite froth obtained. The compositions of the two floats and the residue are shown in Table IV.

TABLE IV

|              | Analysis, percent |       |      |       |                 |                  |
|--------------|-------------------|-------|------|-------|-----------------|------------------|
|              | K                 | Na    | Mg   | Cl    | SO <sub>4</sub> | H <sub>2</sub> O |
| First float  | 17.17             | 1.56  | 5.65 | 2.99  | 40.76           | 31.87            |
| Second float | 15.00             | 2.38  | 5.08 | 6.06  | 34.41           | 37.07            |
| Residue      | 1.83              | 31.35 | 1.04 | 49.83 | 7.59            | 8.36             |

The first float, weighing 199 grams, contained about 97% schoenite and 3% sodium chloride. The second float, weight 62 grams, contained about 72.5% schoenite, 13.8% kainite, 5.5% sodium chloride and 6.8% epsomite. The combined floats, containing about 91.4% schoenite, 3.7% sodium chloride, 3.3% kainite, and 1.6% epsomite, represent a yield of 93% of the schoenite in the feed solids.

The reagent consumption of 600 grams per metric ton of feed solids was the same as in previous examples.

I claim:

1. A process for separating schoenite from salt mixtures containing schoenite and one or more of sodium chloride, epsomite and other magnesium sulfate hydrates, kainite and other impurities which comprises subjecting said mixture, in the form of an aqueous slurry, to a froth flotation separation with a collector comprising a water-soluble petroleum sulfonate having a molecular weight between 300 and 400, whereby to float off a schoenite concentrate.
2. A process according to claim 1, wherein the petroleum sulfonate collector is used in the form of a composition containing of the order of at least 30% of said sulfonate, not more than 50% water, and minor amounts of mineral oils and inorganic salts.
3. A process according to claim 1, wherein the salt mixture is composed of salts containing schoenite and an aqueous brine which is essentially saturated with the water-soluble components of the salt mixture.
4. A process according to claim 1, wherein the mixture of salts is composed of salts from the conversion of kainite to schoenite, or kainite mixed with other salts, and an aqueous liquor obtained from the kainite to schoenite conversion process.
5. A process according to claim 1, wherein the residue from a first flotation is conditioned with additional collector agent and refloated to obtain an increased yield of schoenite.

30

## References Cited

## UNITED STATES PATENTS

|           |        |         |           |
|-----------|--------|---------|-----------|
| 1,765,308 | 6/1930 | Lutz    | 209—166   |
| 2,442,455 | 6/1948 | Booty   | 209—166   |
| 2,596,407 | 5/1952 | Jackson | 209—166 X |
| 3,164,549 | 1/1965 | Seymour | 209—166   |

## FOREIGN PATENTS

574,442 3/1958 Italy.

40 HARRY B. THORNTON, Primary Examiner  
ROBERT HALPER, Assistant Examiner

U.S. Cl. X.R.

252—61